

Patented Sept. 8, 1925.

1,552,610

# UNITED STATES PATENT OFFICE.

NOAK VICTOR HYBINETTE, OF WILMINGTON, DELAWARE.

NICKEL ANODE AND METHOD OF PRODUCING THE SAME, ETC.

No Drawing.

Application filed September 23, 1922. Serial No. 589,995.

To all whom it may concern:

Be it known that I, NOAK VICTOR HYBINETTE, a citizen of the United States, residing temporarily at Wilmington, in the county of New Castle, State of Delaware, have invented certain new and useful Improvements in Nickel Anodes and Methods of Producing the Same, Etc.; and I do hereby declare the following to be a full, clear, and exact description of the invention, such as will enable others skilled in the art to which it appertains to make and use the same.

This invention relates to improved nickel anodes and to a method of producing the same, as well as the improvements in the electrodeposition of nickel therewith.

In my prior application, Serial No. 565,753, filed June 3, 1922, I have described the production of cast anodes by oxidizing molten nickel and casting the anodes from the oxidized nickel. Such oxidized nickel anodes contain from about 0.1% to 0.25% of oxygen and dissolve so readily, when used as anodes in the electrodeposition of nickel, that they cause the bath to become basic.

I have now found that if such an oxidized molten bath is deoxidized, by a suitable deoxidizing agent other than carbon, so as to remove the greater part of the oxygen without completely removing it and rendering the nickel malleable when cast, the anodes made from the resulting bath will be of such solubility that they will dissolve at substantially the same rate at which the nickel is plated on the cathode, so that the bath will remain of correct acidity for long periods of time.

If a molten bath of nickel is reduced or deoxidized by carbon, some carbon monoxide that is formed will be absorbed by the metal, and, when the metal is cast and cooled this gas will give a porous or spongy casting. In order to overcome this sponginess, it has heretofore been attempted to carbonize the metal and subsequently deoxidize it but the desired solubility is thus lost.

I have found, however, that by introducing into the molten metal a suitable deoxidizer which will form a nongaseous oxide, there will be no formation and absorption of gas, and the resulting deoxidized metal can then be cast into anodes which are not spongy or porous in character. The deoxidizing of the nickel, however, is not so

complete that the metal becomes malleable or that it shows more than a small degree of toughness. If the deoxidizer is added in such quantity that the metal becomes malleable or tough, the desired easy solubility is lost. Accordingly, the deoxidized bath is deoxidized without completely removing the oxygen, and I have found that when this is properly done, the resulting metal is ideal for use as anodes for nickel deposition. The anode made of the highly oxidized nickel turns the electrolyte basic, while the fully deoxidized anode turns the electrolyte acid; but where the anode is deoxidized incompletely, according to the present invention, the anode has the correct solubility so that the bath will remain of correct acidity for nickel deposition for long periods of time.

With the ordinary anodes, different electrolytes dissolve the anodes differently, and the chloride bath dissolves the anodes more readily than the sulphate bath; but the anodes of the present invention are almost theoretically perfect in their solubility in the baths commonly used for nickel deposition, so that the new anodes can be used with sulphate electrolytes as well as with chloride electrolytes, etc.

The method of producing the new anodes is illustrated by the following example:

Nickel is melted under oxidizing conditions in a reverberatory furnace preferably lined with ordinary clay brick. The slag formed during the melting down of the nickel may be left on the molten nickel, or it may be skimmed off, or slag ingredients may be added, but at the end of the melting down and slagging operation there should be an oxidized metal covered with a fairly neutral silicate slag. The slag should be one which does not attack or destroy the furnace lining, but otherwise it can be varied in its composition. It should not, however, contain any large amount of nickel, iron, etc., which will react with the deoxidizer used and reoxidize the bath of molten nickel after it has been deoxidized to the proper extent. With careful handling of the furnace, a slag covering of the molten bath may not be necessary, but the danger of reoxidizing the metal and absorbing carbon monoxide is such that the bath can be more readily handled when a layer of slag covers it. After the molten nickel has been oxidized and thereby freed from impuri-

ties, it is subjected to deoxidizing by the addition of a deoxidizer which forms a non-gaseous oxide, care being taken that too much of the deoxidizer is not added. As a deoxidizer, I prefer to use metallic aluminum, since a small excess does not affect the solubility of the anodes. Other deoxidizers may, however, be used, such as magnesium, silicon, manganese or mixture of these with aluminum, etc. The deoxidizer should not however be used in such amount as to affect the desired solubility of the anodes. With an oxidized nickel such as above described I have used from 0.1% to 0.2% of metallic aluminum. The right quantity can be readily ascertained. If from time to time small quantities of the aluminum are added and samples of the molten nickel are taken, it is found that the metal changes in color and grain. By producing a set of samples and having them analyzed and using them for comparison, the proper color and grain of the cast metal can be determined. The correct solubility is obtained when the metal contains between about 0.05% oxygen and 0.05% aluminum. The oxygen is for this purpose determined by dissolving in very dilute nitric acid and determining the nickel in the undissolved residue from which the oxygen is calculated as  $\text{NiO}$ .

After the molten metal has been deoxidized to the desired extent, the metal is poured into molds, care being taken not to introduce any carbonaceous matter. The molds may be metal molds which will rapidly chill the anodes or they may be sand molds in which the metal would cool more slowly.

The new anodes thus produced can be used generally for nickel plating purposes and they enable a good cathode deposit to be produced without the necessity of adjusting the acidity of the bath over long periods of time. When the new anodes are used, it is unnecessary to add salts to the bath. The anodes can also be used with sulphate electrolytes without the addition of chlorides to the bath.

While I do not wish to limit myself by any theoretical explanation of the reason for the remarkable results which the new anodes give, yet I believe that the correct solubility depends not only upon the amount of oxygen, carbon, silicon, etc. that is present, but also upon the grain of the metal. If the grain is fibrous and the metal is tough, the anodes made therefrom are more or less insoluble. If the oxygen is completely removed by the deoxidizing agent, for example, with magnesium, it is possible to have an anode that is malleable and still contains no magnesium; but such an anode does not readily dissolve. In making the new anodes, accordingly, the metal is not completely deoxidized so as to make it malleable and diffi-

cultly soluble, but a small and regulated amount of oxygen is left in the metal such that it has the almost perfect solubility above referred to. Impurities such as copper, iron, etc. are undesirable but may be present in small amount as in ordinary cast anodes, although the nature and amounts of any impurities present should not be such as interfere with the desired solubility of the anodes. When the anodes are produced in the manner above described, the impurities can be almost completely removed during the oxidizing treatment, so that the anodes cast from the molten metal after the incomplete deoxidizing treatment will be of high purity. Where the impurities present in the molten bath are not completely removed in this way they may remain and be present in the cast anodes.

It will thus be seen that the present invention provides new anodes having valuable properties which adapt them for general use in nickel deposition, and with resulting advantages in the nickel deposition such as are unobtainable with any anodes heretofore known, in so far as I am aware. The invention also includes the method of making the new anodes by an oxidizing treatment of the molten bath and a subsequent regulated deoxidizing treatment with a deoxidizer other than carbon, and casting of the resulting metal. The invention also includes the improved method of electrodeposition in which the new anodes are used and which can be carried out with practically automatic regulation of the acidity and without the necessity for the usual adjustments of the acidity of the electrolyte. The electrolytic process in which the new anodes are used is accordingly one of general application with different electrolytes and for different purposes, but is of special application with sulphate electrolytes and without the addition of chlorides, etc. to the bath.

It will be understood that variations and changes can be made in the particular method of making the anodes, as well as in the baths and in the electrodeposition in which the anodes are employed.

I claim:

1. The method of producing nickel anodes which comprises oxidizing a nickel bath, deoxidizing the oxidized bath with a deoxidizer forming a non-gaseous oxide, and casting the deoxidized metal, the deoxidizing of the metal being insufficient to render the metal tough and malleable.
2. The method of producing nickel anodes which comprises melting the nickel, oxidizing the molten nickel, and adding to the oxidized metal a small amount of metallic aluminum insufficient to render the metal tough and malleable, and casting the resulting metal into the anodes.

3. A cast nickel anode having a solubility such that the dissolving of the anode is substantially the same in the common electrolytes and corresponds with the deposit on the cathode with maintenance of the correct acidity of the bath without adjustment.
4. A non-porous cast nickel anode substantially free from impurities and containing about 0.05% of oxygen.
- 10 5. A cast nickel anode comprising incompletely deoxidized oxidized nickel.
6. A nickel anode substantially free from impurities and containing about 0.05% of oxygen.
7. A nickel anode substantially free from 15 impurities and non-malleable.
8. A nickel anode consisting of nickel practically free from carbon, silicon, and oxygen, and non-malleable.
9. A nickel anode substantially free from 20 impurities and containing oxygen in effective amounts but less than .25%.
10. A non-porous, cast nickel anode substantially free from impurities and containing oxygen in effective amounts but less than 25 .25%.

In testimony whereof I affix my signature.  
NOAK VICTOR HYBINETTE.